

Feb. 20, 1951

R. G. RIEDESEL

2,542,058

POLISHING SHEET

Filed Dec. 5, 1949

*Fig. 1*



*Fig. 2*



*Fig. 3*



*Fig. 4*



Inventor

*Richard G. Riedesel*

*By*

*Carpenter, Abbott, Coalter & Kinney*

*Attorneys*

Patented Feb. 20, 1951

2,542,058

# UNITED STATES PATENT OFFICE

2,542,058

## POLISHING SHEET

Richard G. Riedesel, St. Paul, Minn., assignor to  
Minnesota Mining & Manufacturing Company,  
St. Paul, Minn., a corporation of Delaware

Application December 5, 1949, Serial No. 131,072

7 Claims. (Cl. 51—185)

1

This invention relates to coated sheet material having particular utility in the wet polishing of glass, as well as in other polishing operations, and comprising a polishing-powder bonded to the exposed surfaces of resilient particles supported on a flexible backing.

The edges of plate glass panels are commonly ground and polished against steel plates, cork wheels, or felt-covered discs, with loose abrasive or polishing grain being applied continuously as a slurry in water. For the rough grinding, coated abrasive belts capable of operating under constant wetting with water have replaced the systems using loose abrasive grain. Prior to the present invention, however, most if not all of the polishing operations were carried out with fluid suspensions of jeweler's rouge or similar polishing-powders applied to cork, felt, or other polishing-wheels or the like.

My invention provides for more rapid polishing, in fewer passes, than is possible with methods employing loose powders. My invention also avoids the untidiness of these prior art polishing methods. Other advantages will be apparent from the ensuing description of the product.

The several figures of the drawing illustrate, in side elevation, various specific embodiments of my invention.

The embodiment of Figure 1 includes a flexible backing member 10 coated with a sizing coat 11 and carrying a layer of resilient particles 12 held in place by a first adhesive binder 13. The upper surface of the particles and the interposed binder is further coated with a polishing layer 14 consisting of polishing-powder dispersed throughout an adhesive binder having somewhat greater firmness and hardness than the first binder coat 13.

In the modification shown in Figure 2, a flexible backing member 20 is coated directly with an adhesive binder 23 into which are pressed the resilient particles 22. The particles 22 and adhesive layer 23 are then coated with a layer of adhesive binder 25 and a final covering of polishing powder 26.

Figure 3 shows a modification in which each resilient particle 32 is first separately encased in a hardened coating 34 of a mixture of polishing-powder and adhesive, and is then bonded to the flexible backing 30 by means of an adhesive binder layer 33.

In Figure 4, the resilient particles 42 are bonded to the flexible backing 40, previously covered with a sizing coat 41, by means of an adhesive binder

2 coat 44 consisting of a dispersion of polishing powder in an adhesive binder.

One specific example of a polishing-sheet made as indicated in Figure 1 and which has given excellent results in the wet polishing of glass when used in the form of a continuous belt will now be described. While endless belts are preferred, it will be apparent that my sheet material has utility also in the form of discs, cones, flat sheets or strips, etc.

The flexible backing layer was prepared from stretched pre-shrunk drill cloth having a thread count of 76 x 48 and weighing about 50 grains per 24 sq. in. The cloth was first impregnated with a 20% solution of 20 C. P. S. (47-50% ethoxy) ethyl cellulose in a mixture of xylol and ethylene glycol monoethyl ether, and after drying was found to contain about 15-17 grains per 24 sq. in. of the dry residue. During drying, the web was held in a flat stretched condition. The ethyl cellulose stiffened the fabric, provided water-resistance, and improved the anchorage while reducing the penetration of the sizing coat.

The sizing coat consisted of 85 parts of polyvinyl acetate ("Vinylite AYAT"), and 11 parts of diatomaceous earth, in 148 parts of xylol and 148 parts of alcohol. Sufficient of the solution was applied to provide 10-12 grains/24 sq. in. of the solids after drying. This sizing coat further improved the water-resistance and non-stretching properties of the web, and also provided improved anchorage for the adhesive binder.

A drying-oil-modified alkyd resin was used as the binder for the resilient particles. Suitable binders are those previously employed in the coated abrasives industry for bonding abrasive grit to fabric backings: cf. Guth Patent No. 2,202,765. One specific alkyd resin binder which has given good results in the present invention is a linseed-oil-modified phthalic glyceride. By its use, the resilient particles are firmly and resiliently bonded to the sized backing. About 25-30 grains/24 sq. in. of this binder, on the solvent-free basis, is used.

As the resilient particles, I prefer to employ cork particles. The comminuted cork is preferably screened to remove off-size lumps and fines, the portion corresponding approximately to screen sizes of 24-36 mesh being retained in the present example, although other particle sizes may be used. This material is spread over the adhesive-coated sheet and pressed down with rollers, the excess then being shaken off. Substantially a single thickness of particles is ordinarily obtained where the binder weight and the

particle size are as specified, the weight of the layer of cork particles being approximately 9-10 grains/24 sq. in. The sheet is then placed in an oven for 24 hours, to remove the solvent and to cure the binder.

The sheet is now ready for application of the polishing layer, which in this case is a mixture of "air-float tripoli" (siliceous polishing-powder) and phenolic resin varnish, 75 parts by weight of the tripoli being mixed into enough liquid varnish to provide 29 parts by weight of non-volatile components. The coating weight of this mixture, on the dry basis, is 104 grains per 24 sq. in. Further heating of the coated sheet cures the varnish binder to a hard and tough state.

Endless belts may be made from the coated and cured sheet material by slitting to proper width, and skiving and splicing together the ends of a section of desired length, in accordance with well-known practice. The resulting belt retains its shape and strength when operated under a constant stream of water. It reduces rough-ground glass edges to a smooth polished condition rapidly and efficiently. For example, plate glass rough-edged with grit 320 abrasive belt was finished to the desired high polish by the action of the polishing-belt as above described, operating under a constant stream of water, in less than 5 seconds. Prior art methods of finishing, using a slurry of powder and water, would have required at least several minutes to produce an equally acceptable edge.

Thus my novel sheet material provides for increased speed and efficiency of polishing. An additional and unexpected advantage is the long service life of these polishing-belts. Cork is quite friable, and under the severe pounding experienced in wet grinding would be expected to shear or break off, or to pull away from the binder, after only a few passes across the work-piece. On the contrary, however, I have discovered that the presence of the cork particles improves both the service life and the polishing speed and efficiency of such belts, as well as the quality of the finish produced. For example, a belt made with the same mixture of tripoli and varnish, coated directly on the treated and sized cloth backing but in the absence of the cork particles, produced scratches in the glass edge and was no longer effective after only 5 minutes of service. In contrast, the belt having a layer of cork particles and made in accordance with the foregoing example produced a scratch-free finish and was still useful after one hour of operation. Furthermore my cork-containing belt was easier to handle, the layer of cork and binder making the strip less limp and more water-resistant.

In probable partial explanation of the superior results obtained with my novel sheet material, the following suggestions are offered. The presence of the resilient mass beneath the polishing powder maintains a more nearly constant pressure of all operative powder particles against the surface to be polished, hence a maximum polishing effect is obtained, and somewhat coarser powders may be employed than would otherwise be applicable because of a tendency toward scratchiness. The unevenness of the polishing surface, caused by the presence of the underlying relatively large particles of cork, increases the unit pressure against the workpiece and makes for faster cutting. Placing the polishing-powder in close proximity to the resilient cork particles emphasizes the yielding qualities of the

base while still permitting the use of a hard, firm binder for getting the maximum cutting efficiency from the powder. The cork particles themselves aid in burnishing and improving the polish of the work-piece.

Regardless of the particular reasons and mechanisms involved, the fact remains that actual tests have shown my novel polishing-sheet, particularly in the form of endless belts on a wet-sanding machine, to provide faster, more efficient, more economical, and generally superior industrial polishing of the edges of glass panels and other surfaces than has been possible by means of previously employed systems.

It will be apparent from Figures 2-4 that a number of alternative structures may be employed. Figure 2, for example, illustrates a sheet in which the sizing coat of Figure 1 is eliminated, and the polishing-powder is applied as a separate dry coating to the outer binder layer prior to drying and curing the same. In this construction, the backing is preferably more completely filled with the ethyl cellulose or equivalent impregnating material, and in most instances a somewhat larger amount of adhesive binder for the resilient particles is applied in order still further to impregnate the adjacent surface of the backing. The outer binder layer may be somewhat lighter than that of the construction shown in Figure 1, and the total amount of polishing-powder will then be reduced also. However, all of the powder will be at, or very close to, the surface of the sheet and hence at a position of maximum effectiveness.

In Figure 3 the cork particles are individually completely surrounded by, or encased in, a shell of the mixture of polishing-powder and binder, and the encased particles are bonded directly to the impregnated backing by means of an additional amount of a somewhat softer type of adhesive binder. Only one binder coat on the sheet material, and only one oven treatment, is required for this structure.

Figure 4 illustrates another modification in which a single binder coat is sufficient. In this case, the single binder composition carries both the resilient particles and the polishing-powder.

It will be apparent, in view of the description, that many other combinations, to provide analogous advantages, are possible, and such combinations and variations are contemplated as coming within the scope of the appended claims.

Additionally, many other equivalent materials and components will be apparent to those familiar with the art, in view of the teachings here provided, and such elements are also contemplated.

Cloth backings have also been successfully impregnated with polystyrene resin or polyvinyl butyral resin in place of ethyl cellulose. Suitable papers or other fibrous webs having the required strength and dimensional stability may replace the fabric. Vulcanized fiber, and various resinous or polymeric films, may replace the impregnated fibrous web here specified as the backing member.

In place of vinyl acetate polymer, plasticized phenolic resins have been employed as the sizing coat 11 of Figure 1; and polyvinyl butyral resin was then used to replace the alkyd resin binder 13 and the binder of the polishing layer 14. In another example, a drying oil modified phenol-aldehyde resin as the binder for the polishing-powder provided excellent results. One specific formula of this type employs a varnish compris-

ing one part of para-phenyl-phenol: formaldehyde resin ("Bakelite BR-254") and three parts of dicyclopentadiene-modified linseed oil ("75-5" oil), applied from solution in xylol and naphtha. Polyvinyl butyral modified with minor proportions of phenolic resin has also been used. These and other similar film-forming adhesive materials are all found to have desirable qualities. Much softer materials are to be avoided, however, because of their lack of required strength; and much harder materials, e. g. combinations of polyvinyl butyral with an excessively high proportion of phenol-aldehyde resin, are undesirable since they may cause scratching of the work-surface in some cases.

The various combinations of impregnants, sizes, and binders hereinabove noted have been found to provide particularly desirable results in combination with cork particles and tripoli polishing-powder for polishing glass edges. The relatively hard outer binder adheres firmly to the cork particles and the surrounding somewhat softer inner binder, which in turn adheres well to the cork and to the sizing layer where such is used, or directly to the impregnated fibrous backing as indicated in Figure 2, to provide a well-unified composite sheet. For polishing other classes of materials, still other combinations are found suitable. Thus, a sheet such as indicated in Figure 4 was found to be excellent for polishing resinous panels such as methyl methacrylate polymer ("Lucite") when made with a cloth backing impregnated with polyvinyl butyral resin and primed with a heat-setting phenol-aldehyde resin applied from solution in water, alcohol and ethylene glycol monoethyl ether, and with a polyvinyl butyral resin binder for the cork particles and the mineral polishing-powder. In this case, an iron oxide polishing-powder was used.

Air-float tripoli, a finely divided silica polishing-powder, combines rapid cutting action with excellent polishing action when used in these novel polishing-sheet structures for such applications as the polishing of glass, even though under ordinary lapping usage, such powder is considered to be too coarse for final polishing. Pumice powder of 3F or 4F grade is also satisfactory. Materials such as polishing grades of tin oxide, cerium oxide, or iron oxide are much slower and, for my purposes where the polishing of glass is concerned, are needlessly fine. These are the classes of polishing-powders ordinarily required to be used in commercial polishing operations on glass, in order to avoid scratching of the glass surface.

As the resilient particles, I greatly prefer to employ cork particles, since, as previously mentioned, these provide an additional burnishing action in addition to a particularly advantageous degree of compressibility and resiliency. Furthermore, my preferred binder compositions adhere well to the cork particles. However, I have successfully used such alternative particulate materials as vulcanized rubber particles; and other natural or synthetic compressible and resilient materials having substantially the resiliency of my preferred cork particles, together with adequate water-resistance, heat-resistance, etc., may also be used.

Having now described various embodiments of my invention for purposes of illustration, but without intent to be limited thereto, what I claim is as follows:

- 5 1. A polishing-sheet suitable for the polishing of glass edges, comprising a flexible, dimensionally stable backing, a series of resilient protuberances over one surface thereof, and a polishing-powder uniformly adherently bonded to the outer surfaces of said protuberances.
- 10 2. A polishing-sheet suitable for polishing of glass edges, comprising a flexible, water-resistant, dimensionally stable backing, a layer of cork particles adherently bonded to one surface thereof, and a mineral polishing-powder uniformly adherently bonded to the outer surfaces of said particles.
- 15 3. A polishing-sheet suitable, in the form of an endless belt, for wet-polishing of glass edges, comprising a flexible, water-resistant, dimensionally stable backing, a layer of cork particles adherently bonded to one surface thereof, and a mineral polishing-powder surrounding each cork particle and adherently bonded thereto.
- 20 4. A polishing-sheet suitable, in the form of an endless belt, for wet-polishing of glass edges, comprising a flexible, water-resistant, dimensionally stable backing, a layer of cork particles adjacent one surface thereof, and an adhesive
- 25 30 containing uniformly admixed polishing-powder, said binder surrounding each cork particle and adherently bonding said particles to said backing.
- 35 5. A polishing-sheet comprising, in order, a flexible, water-resistant, dimensionally stable impregnated fibrous backing, an inner adhesive binder layer, a layer of resilient particles, and an outer adhesive binder layer containing a mineral polishing-powder, each successive layer being firmly bonded to the previously-named layer.
- 40 6. A polishing-sheet comprising in order a flexible, water-resistant, dimensionally stable backing comprising a porous fabric base impregnated with a flexible water-resistant film-forming polymer and surface-sized with a flexible water-resistant film-forming polymer, an inner resinous adhesive binder layer, a layer of resilient particles, and an outer resinous binder and polishing layer comprising a mineral polishing-powder uniformly distributed throughout a varnish binder, each successive layer being firmly bonded to the previously-named layer.
- 45 7. A polishing-sheet comprising in order a flexible, water-resistant, dimensionally stable backing comprising a porous cloth impregnated with a water-resistant, film-forming cellulose polymer composition, a surface sizing of a film-forming vinyl polymer composition, an inner alkyd resin adhesive binder layer, a layer of resilient cork particles of about 24-36 mesh size, and an outer binder and polishing layer composed of mineral polishing-powder uniformly distributed throughout a phenolic resin-drying oil varnish, each successive layer being firmly bonded to the previously-named layer.

RICHARD G. RIEDESEL.

No references cited.